

## UNITED STATES PATENT OFFICE

1,926,768

## PREPARATION OR SIZE FOR SILK, ARTIFICIAL SILK OR OTHER FIBER

Auguste Firmin Galvin, Lyon, France

No. Drawing. Application June 25, 1926, Serial No. 118,612, and in France July 4, 1925

1 Claim. (Cl. 134—18)

This invention relates to an improved sizing preparation for textile fibers and more especially for silk or artificial silk fibers, which facilitates subsequent operations, of the type employing a refined drying oil or light varnish.

The object of the invention is the formation of a sizing preparation which is substantially non-acid in its composition and hence will not burn or damage the fibers being treated when applied thereto, and one which is soluble in the solvent used for removing the size from textiles, and hence can be completely removed in the degreasing or boiling operations which accompany the dyeing.

Known processes based on the employment of boiled linseed oil do not possess these advantages. In practice after a certain time silk so treated sticks together and turns strongly yellow or is not completely desized for dyeing. These disadvantages arise from the use of metallic dryers, litharge, manganese compounds or the like being employed alone or in combination and to the extent of 4 to 7% of the weight of the oil. After boiling these dryers render the oil acid and turn it brown, nearly to a dark maroon color, the acidity tending to burn the silk and the color preventing the forming of a clear liquid.

According to the invention a drying preparation for use in the preparation of a size for textile fibers comprises cobalt acetate, cobalt oleate or cobalt resinate mixed with linseed oil and boiled and then added to a refined oil or extra light varnish.

The following is an example of a drying oil produced in accordance with the invention.

25 grams of a dryer such as cobalt acetate, cobalt oleate or cobalt resinate are mixed with 200-500 grams of linseed oil, the mixture being then boiled and added to 100 kilograms of refined oil or extra light varnish or 150 grams of cobalt acetate, cobalt oleate or cobalt resinate in the form of a stiff paste, are added to the 100 kilograms of refined oil. These quantities may be lessened if desired. The dryer may be mixed with the oil either hot or cold.

By cobalt resinate is meant the product obtained by treating acetate salts of cobalt with resins at a high temperature.

By a suitable refined oil or extra light varnish is meant an oil of the kind employed in the printing industry such oils being in general commercial use. These oils are linseed oil, boiled without litharge, manganese or other dryers, the difference between their viscosities being due to the amount of boiling which they have undergone.

In this way a drying preparation is obtained which is practically non-acid from the fact that it contains only a very small quantity of dryer which will not burn the silk. This oil is but very slightly colored having merely a champagne tint which enables a very clear liquid to be obtained.

The acidity of the bath and the dark color of ordinary linseed oil given by an ordinary dryer is diminished by adding five and a half parts of refined oil or extra light varnish without dryer for each part of ordinary boiled linseed oil.

In this way the quantity of acid is six and a half times less and the dark color is cleared and approaches that of refined oil. The mixture may be made hot or cold.

The composition and proportions of the constituents of the sizing bath can be varied to a certain degree according to the nature and state of the threads to be treated and to the type of finish it is desired to obtain, either lustrous or otherwise. The following example is found to give a good result.

|                                          |       |                   |
|------------------------------------------|-------|-------------------|
| Petrol or benzine                        | 2,000 | cubic centimeters |
| A drying oil produced as above described | 1,000 | cubic centimeters |
| Crude ordinary China wood oil            | 500   | cubic centimeters |
| Soap, benzine, light mineral oil         | 100   | cubic centimeters |
| Petroleum jelly or olive oil             | 100   | cubic centimeters |
| Grease, lanoline or tallow               | 30    | grams             |
| Wax                                      | 30    | grams             |

If a very pliable size is required the China wood oil is omitted and the proportion of petrol or benzine reduced to 1300 cubic centimeters.

If ordinary dryers, that is an oil treated or boiled with litharge or manganese are added, in addition, only one sixth or one ninth of the amount normally employed is used and the acidity of this small quantity is neutralized by the presence of the olive oil and tallow, thus only 650 grams would be boiled with three litres of linseed oil. The refined oil and dryer can be mixed hot or cold.

The linseed oil, cobalt acetate, cobalt oleate or cobalt resinate are first mixed together, then cooked. It is only after cooking that they are added to the refined oil or extra light varnish.

By refined oil is understood an oil of the kind used in the printing industry. Such oils are usually used right along in commerce. A printing oil is a linseed oil cooked without siccative, that is, in the absence of all products such as for example litharge or manganese, or other siccative.

According to whether this linseed oil is more

or less cooked, it is called: refined oil or extra light varnish, light, strong, extra strong, etc.

When linseed oil is cooked only a little, it is called refined oil; when it is cooked more, it is called extra light varnish; when it is cooked more, it is called weak or light varnish; when it is cooked still more, it is called mediocre varnish; by increasing the cooking, a strong varnish is obtained; by increasing the cooking still more, an extra strong varnish is obtained which presents a very thick aspect (like glue).

In treating certain delicate silks or for obtaining a very strong sizing a first thin coat is applied of stiff glue, dextrine, casein, baked starch, 15 gelatine or a gum.

This first sizing prevents the thread from having the oil dryer applied directly thereon.

In certain cases after sizing the fabric may be treated in a softening bath of either olive oil, 20 castor oil or mineral oil or of benzine soluble soap, grease, lanoline, tallow or dilute Japan wax in petrol or benzine.

In a light softening bath, color of any shade

can be added according to the shade desired for the sizing.

Treatment is effected by immersing the material in the sizing bath the time varying according to the nature, from five to thirty minutes. 80

After treatment the material is hung in the air to dry and then dried in a warm chamber kept at a temperature below 45° C.

The treatment is similar for softening to that for sizing. 85

What I claim as my invention and desire to protect by Letters Patent is:—

A substantially non-acid strengthening adhesive size for textile fibers which is soluble in the alkaline solvent used for removing size from textiles, comprising a boiled mixture of cobalt drier and linseed oil in substantially the proportions of from 200 to 500 grams of linseed oil and substantially 25 grams of cobalt drier and 100 kilograms of boiled linseed oil free from 90 driers. 95

AUGUSTE FIRMIN GALVIN.

25

100

30

105

35

110

40

115

45

120

50

125

55

130

60

135

65

140

70

145

75

150